

J. M. BOTTUM

Annealing Metals.

No. 96,874.

Patented Nov. 16, 1869.

Fig. 2.



Fig. 1.



Witnesses.

W. B. Deming  
John Gunnell

Inventor:

J. M. BOTTUM  
by Knight Berg  
Attorneys

# UNITED STATES PATENT OFFICE.

JAMES M. BOTTUM, OF NEW YORK, N. Y.

## IMPROVED PROCESS OF AND APPARATUS FOR ANNEALING METALS.

Specification forming part of Letters Patent No. **96,874**, dated November 16, 1869.

*To all whom it may concern:*

Be it known that I, JAMES M. BOTTUM, of the city, county, and State of New York, have invented a new and useful Improvement in Annealing Metals; and I do hereby declare that the following is a sufficiently full, clear, and exact description thereof to enable one skilled in the art to which my invention appertains to carry it into effect, reference being had to the accompanying drawings, which form part of this specification.

In carrying out my invention I employ an annealing-pot of any common or suitable form, within which the metal to be annealed may be packed in charcoal or other material and the whole introduced into the furnace for heating, in customary manner. When the heating is completed the pot is removed from the furnace and placed in my improved cooling-chamber, which is then closed air-tight, until the gradual cooling of the metal within the annealing-pot is finished. The annealing-pot, during this process, is supported at a considerable distance from the external walls of the chamber, and the cooling-chamber itself is preferably supported in such a manner as to lessen or avoid any unequal conduction of heat from its various parts. If the cooling-chamber be of large size, it will be lined on the interior with fire-brick or other non-conducting material, and will be furnished with rails, on which may run a truck to carry the annealing pot in or out. The door of the cooling-chamber may be hung on hinges and its joints packed with charcoal or other proper material, so as to render the tight clamping of the cover upon the chamber unnecessary.

To illustrate the invention, I will proceed to describe the simple form thereof, which is represented in the accompanying drawings.

Figure 1 represents a longitudinal section of the cooling-chamber, and Fig. 2 a transverse section of the same, each figure showing an external view of the annealing-pot within the chamber.

Similar letters of reference indicate corresponding parts in both views.

A represents an annealing-pot, made in cylindrical or other common form, and provided with a removable head or cover, which may be held down by wires *a a*.

B represents a hollow base, supporting the cooling-chamber C, which may be of cylindrical or other form, and is provided with a removable head, D, packed or luted, as shown at *d*, and held securely to its seat by knuckle-bolts E and nuts F.

An air cock or valve, G, is employed to permit the escape of the air displaced by heat or by gases evolved within the chamber, the said valve being then immediately closed to prevent any reflux of air until the cooling operation is completed, and then reopened, so as to relieve the head D of unequal pressure on the outside when it is to be removed for the purpose of taking out the annealing-pot. For special kinds of work, or when from any cause a more perfect vacuum is required within the chamber, the air is exhausted by means of an air-pump applied to the cock G.

In the illustration here given the pot A is supported within the chamber G by a frame or stand, which may consist of two or more horizontal rods, H H, set at their ends in cross-bars I I, so that the pot will have no direct contact with the walls of the chamber, but will be surrounded on all sides by gas. The effect of this provision is to prevent the rapid or unequal cooling of the pot or its contents, and the entire apparatus effectually protects the metal under treatment from any injurious atmospheric contact, any oxygen which may be inclosed within the chamber C being speedily consumed by contact with the red-hot box or pot A.

I claim and desire to secure by Letters Patent—

The process and apparatus for annealing metals, substantially as herein described.

JAMES M. BOTTUM.

Witnesses:

W. B. QUINN,  
J. C. BUCKINGHAM.